

## UNITED STATES PATENT OFFICE

2,371,623

METHOD OF PRESERVING SOAP AND  
RESULTING PRODUCT

Lloyd F. Henderson, Reading, Mass., assignor to  
Lever Brothers Company, a corporation of  
Maine

No. Drawing. Application February 6, 1943,  
Serial No. 475,001

14 Claims. (Cl. 260—398.5)

The present invention relates to detergent compositions derived from higher fatty materials and, more particularly, to soap and non-soap products comprising one or more ingredients which are susceptible to deterioration and the development of rancidity. In accordance with the present invention, it is possible to inhibit or retard this deterioration by incorporating in the detergent a small quantity of one or more of the group of stabilizing substances herein disclosed.

It is an advantage of this invention that the stabilizing substances which it is proposed to incorporate in the detergent do not have the property of imparting undesirable odors or of causing discoloration of the detergent as is frequently the case when stabilizers, for example, phenolic compounds are utilized for stabilizing purposes. Moreover, the group of stabilizing substances used in accordance with the present invention are water soluble and do not form precipitates as is sometimes the case when certain metallic compounds are used. Furthermore, the present stabilizing substances may be utilized in comparatively small amounts based on the weight of the detergent whereby the amount of detergent in the product is not appreciably decreased, the physical characteristics of the detergent, for example, with respect to hardness, are not adversely affected, and the cost of stabilizing the detergent is kept at a minimum.

By "higher fatty detergent" I refer to soaps and non-soaps having an aliphatic radical of 8 or more carbon atoms. The soaps are the alkali metal, ammonium, alkyl, amine and alkylolamine salts or esters of higher fatty acids such as may be prepared, for example, by saponifying an animal or vegetable fat with an alkali metal compound. The higher fatty non-soap detergents are sulfonated or sulfated compounds such as higher alkyl sulfonates or sulfates, taurides, and other compounds derived from higher fatty materials which group is well known in the art as having detergent properties. All compositions of this type, regardless of the source of the ingredients or the technique of manufacture, may be stabilized in accordance with the present invention and all such compositions are intended to be within the scope of the invention. For convenience only, I will describe my invention hereinafter as applied to soap.

It is well known that soaps of the character described turn rancid as a result of oxidation or otherwise. In the case of white soap there is usually a noticeable discoloration. It is an object of this invention to inhibit or retard this tendency

to develop rancidity without at the same time incorporating large amounts of non-soap materials into the soap and without causing undesirable collateral effects such as the development of undesirable color and odor, and softness.

The susceptibility to the development of rancidity which is characteristic of conventional soaps may be inhibited or retarded in accordance with this invention by incorporating one or more of the group of stabilizing substances herein disclosed, in the soap at any convenient stage of the soap making process. Preferably, the stabilizing substances are added to the soap subsequent to its boiling, for example, during crutting or milling, or both. The exact time at which the stabilizing substances are added or the method by which they are added to the soap is not critical, and by the term "incorporated in the soap" it is intended to include all such variations in technique as might suggest themselves to one skilled in the art.

It is an advantage of the invention that it is necessary to use only relatively small amounts of the stabilizing substances in order to effect adequate stabilization. As a result, the percentage of actual soaps in the product need not be materially reduced, and the physical characteristics of the soap such as its hardness are not appreciably affected. For example, adequate stabilization may be afforded by the use of a small amount of stabilizer of the order of 0.01 to 1.0% based on the weights of the soap and, in general, less than 0.5% of stabilizer in the soap product is desirable for adequate stabilization. There is no apparent advantage in utilizing greater amounts of the stabilizer, and, therefore, it is preferred to utilize amounts within the above range, although amounts up to not more than about 5% of stabilizer, based on the weight of the soap, may be employed.

The group of stabilizing substances which may be used in accordance with the invention are any of the aliphatic or aromatic compounds containing one or more trivalent nitrogens and two or more carboxyl groups connected to at least one of the nitrogens through a short aliphatic chain having not more than four carbon atoms and preferably through the methylene group. Such compounds would contain the essential group:

50



where X is the above referred to short aliphatic chain, such as  $-\text{CH}_2-$ . The following general

formulas are illustrative of the type of compounds above defined:



in which X is a short aliphatic or substituted aliphatic chain;  $X^1$  is a hydrogen, alkyl, cycloalkyl, aryl, or substituted alkyl, cycloalkyl or aryl group, or a carboxyl alkyl group containing not more than 4 carbon atoms in the chain portion of the molecule; Y is an aliphatic or substituted aliphatic chain, or an aromatic or cycloaliphatic nucleus. The carboxylates, including the salts of the above acids, such as alkali metal, ammonium, and amine salts, and the esters of the acids, such as the methyl and ethyl esters, as well as the anhydrides of the acids, are equally effective and are included within the above definition. When a carboxylate is used as the stabilizer the positive radical of the carboxylate preferably may be the same as the positive radical of the detergent. Thus, an ammonium salt of one of the above acids would be used with an ammonium soap.

Among the compositions of this type which may be used in accordance with this invention are the alkali metal salts of, for example, the following:

Nitrilotriacetic acid  
Alkylene diamino tetracetic acid  
C-alkyl-nitrilotriacetic acid  
C-diethyl-nitrilotriacetic acid  
C-phenyl-nitrilotriacetic acid  
C-phenyl alkyl-nitrilotriacetic acid  
C-cyclohexenyl-nitrilotriacetic acid

The above list of compounds is given merely by way of illustration and is not intended to be understood as limitative of the scope of the invention.

The nitrilotriacetic acid radical referred to in the specification and the claims has the following formula:



Nitrilotriacetic acid as the formula:



Ethylene diamino tetracetic acid has the following formula:



In order to illustrate the effectiveness of the above group of stabilizing compounds, the following tests, which are given merely by way of example, were carried out with a substantially neutral kettle soap prepared by saponifying substantially 70 parts tallow and 25 parts coconut oil with sufficient caustic soda to make a neutral

soap. Samples of the resulting soap and additional samples thereof prepared by adding small quantities of the stabilizing compounds during crutching were then permitted to stand at room conditions and also under controlled conditions of elevated temperature and high humidity. At the end of each day the soap was examined and any odor indicative of rancidity was noted. The following table (Table I) of the results obtained with specific samples is given merely by way of illustration and is not to be understood as limiting the scope of the invention.

Table I

| 15 | Stabilizing compound                  | Amount of stabilizing compound | Duration of test period |
|----|---------------------------------------|--------------------------------|-------------------------|
|    |                                       |                                | 115° F. 80% R. H.       |
| 20 | Nitrilotriacetic acid.....            | 0.2                            | Rancid after 79 days.   |
|    | Ethylene diamino tetracetic acid..... | 0.2                            | Good after 247 days.    |
|    | Blank.....                            | None                           | Rancid after 3 days.    |

The duration of the test period in the above table indicates the period during which the soap had remained stable and did not develop rancidity. Thus it is shown that the incorporation of a small amount of a stabilizing compound selected in accordance with the invention has an exceptionally strong stabilizing action against the development of rancidity.

The above specific test results are indicative of the stabilizing effect attained with a framed type of soap. Similar results were obtained in tests directed to a milled type of soap. In carrying out these additional tests, soap chips of reduced moisture content were prepared in a conventional manner utilizing the kettle soap stock referred to above. Sample amounts of the dried chips were then milled alone and with a small amount of a stabilizing compound added during the milling, following which the soap was plodded and formed into cakes. The soap was then tested for stability against the development of rancidity as described above. The following table (Table II) of the results obtained with specific samples which is given merely as illustrative, indicates that even superior results were obtained in the case of a milled soap as compared with a framed type of soap.

Table II

| 55 | Stabilizing compound                  | Amount of stabilizing compound | Duration of test period |                     |                       |
|----|---------------------------------------|--------------------------------|-------------------------|---------------------|-----------------------|
|    |                                       |                                | 115° F.<br>80% R. H.    | 95° F.<br>50% R. H. | Room temper-<br>ature |
| 60 | Nitrilotriacetic acid.....            | 0.2                            | Rancid 46 days.         | Good 202 days.      | Good 202 days.        |
|    | Ethylene diamino tetracetic acid..... | 0.2                            | Good 224 days.          | Good 224 days.      | Good 224 days.        |
|    | Blank.....                            | None                           | Rancid 3 days.          | Rancid 13 days.     | Rancid 64 days.       |

In view of the above data (Tables I and II), it is apparent that stabilizing compounds selected from the group herein disclosed possess marked stabilizing properties when incorporated in soap. Similar test results may be obtained by the use of compounds selected from the group herein disclosed other than those whose test results have been specifically set forth in the tables above for illustrative purposes and the use of all such compounds in a soap composition is intended to be within the scope of the present invention.

I claim:

1. A detergent selected from the group consisting of soap and higher fatty non-soap detergents having a normal tendency to become rancid and being rendered resistant to the development of rancidity by having incorporated therein a small amount of a non-detergent compound selected from the group consisting of aliphatic and aromatic compounds containing at least one trivalent nitrogen and at least two carboxyl groups connected to at least one of the nitrogens through a short aliphatic chain having not more than four carbon atoms, and their salts, esters and anhydrides.
2. A detergent selected from the group consisting of soap and higher fatty non-soap detergents having a normal tendency to become rancid and being rendered resistant to the development of rancidity by having incorporated therein a small amount of the order of about 0.01 to 1.0%, based on the weight of the detergent, of a non-detergent compound selected from the group consisting of aliphatic and aromatic compounds containing at least one trivalent nitrogen and at least two carboxyl groups connected to at least one of the nitrogens through a methylene group, and their salts, esters and anhydrides.
3. A soap rendered resistant to the development of rancidity having incorporated therein not more than 5% of an alkali metal salt of an organic aminocarboxylic acid containing at least one nitrilodiacetic acid radical.
4. A soap rendered resistant to the development of rancidity having incorporated therein a small amount of the order of about 0.01 to 1.0% of an alkali metal salt of nitrilotriacetic acid.
5. A soap rendered resistant to the development of rancidity having incorporated therein a small amount of the order of about 0.01 to 1.0% of an alkali metal salt of ethylene diamino tetracetic acid.
6. A method of retarding the development of rancidity of a detergent selected from the group consisting of soap and higher fatty non-soap detergents having a normal tendency to become rancid, comprising incorporating in said detergent a small amount of a non-detergent compound selected from the group consisting of aliphatic and aromatic compounds containing at least one trivalent nitrogen and at least two carboxyl groups connected to at least one of the nitrogens through a short aliphatic chain having not more than four carbon atoms, and their salts, esters and anhydrides.
7. A method of retarding the development of rancidity of a detergent selected from the group consisting of soap and higher fatty non-soap detergents having a normal tendency to become rancid, comprising incorporating in said detergent a small amount of the order of about 0.01 to 1.0% based on the weight of the detergent of a non-detergent compound selected from the group consisting of aliphatic and aromatic compounds containing at least one trivalent nitrogen and at least two carboxyl groups connected to at least one of the nitrogens through a methylene group, and their salts, esters and anhydrides.
8. A method of retarding the development of rancidity of a soap comprising incorporating in the soap not more than 5% of an alkali metal salt of an organic aminocarboxylic acid containing at least one nitrilodiacetic acid radical.
9. A method of retarding the development of rancidity of a soap comprising incorporating in the soap a small amount of the order of about 0.01 to 1.0% of an alkali metal salt of nitrilotriacetic acid.
10. A method of retarding the development of rancidity of a soap comprising incorporating in the soap a small amount of the order of about 0.01 to 1.0% of an alkali metal salt of ethylene diamino tetracetic acid.
11. An alkali metal soap having a normal tendency to become rancid and being resistant to the development of rancidity by having incorporated therein not more than 5% of a non-detergent compound selected from the group consisting of aliphatic and aromatic compounds containing at least one trivalent nitrogen and at least two carboxyl groups connected to at least one of the nitrogens through a short aliphatic chain having not more than four carbon atoms, and their salts, esters and anhydrides.
12. An alkali metal soap having a normal tendency to become rancid and being rendered resistant to the development of rancidity by having incorporated therein a small amount of the order of about 0.01% to 1.0%, based on the weight of the soap, of a non-detergent compound selected from the group consisting of aliphatic and aromatic compounds containing at least one trivalent nitrogen and at least two carboxyl groups connected to at least one of the nitrogens through a methylene group, and their salts, esters and anhydrides.
13. A method of retarding the development of rancidity in alkali metal soaps having a normal tendency to become rancid, which comprises incorporating in the soap not more than 5% of a non-detergent compound selected from the group consisting of aliphatic and aromatic compounds containing at least one trivalent nitrogen and at least two carboxyl groups connected to at least one of the nitrogens through a short aliphatic chain having not more than four carbon atoms, and their salts, esters and anhydrides.
14. A method of retarding the development of rancidity in alkali metal soaps having a normal tendency to become rancid, which comprises incorporating in the soap a small amount of the order of about 0.01% to 1.0%, based on the weight of the soap, of a non-detergent compound selected from the group consisting of aliphatic and aromatic compounds containing at least one trivalent nitrogen and at least two carboxyl groups connected to at least one of the nitrogens through a methylene group, and their salts, esters and anhydrides.

CERTIFICATE OF CORRECTION.

Patent No. 2,371,623.

March 20, 1945.

LLOYD F. HENDERSON.

It is hereby certified that error appears in the printed specification of the above numbered patent requiring correction as follows: Page 1, first column, line 7, for "th s" read --this--; page 2, first column, line 57, for "acid as" read --acid has--; line 74, for "70 parts" read --75 parts--; and second column, line 20, Table I, third column thereof, for the indistinct numeral before "days" read --247--; and that the said Letters Patent should be read with this correction therein that the same may conform to the record of the case in the Patent Office.

Signed and sealed this 5th day of June, A. D. 1945.

Leslie Frazer

(Seal)

Acting Commissioner of Patents.